

Feb. 15, 1927.

E. R. MILLS ET AL

1,617,604

METHOD OF MAKING FABRIC FOR CORSETS, BANDEAUX, BRASSIERES, AND THE LIKE

Filed June 25, 1924



Fig. 2.

Fig. 1.

Fig. 4.



Fig. 3.



Inventors  
Ernest R. Mills  
Carl J. Hazelton  
By attorney  
Samuel G. Bowditch.

Witness  
C. F. Mason.

Patented Feb. 15, 1927.

1,617,604

# UNITED STATES PATENT OFFICE.

ERNEST R. MILLS AND CARL J. HAZELTON, OF WORCESTER, MASSACHUSETTS.

METHOD OF MAKING FABRIC FOR CORSETS, BANDEAUX, BRASSIÈRES, AND THE LIKE.

Application filed June 25, 1924. Serial No. 722,390.

This invention relates to a method of manufacturing fabric for use in making elastic garments in the nature of corsets, bandeaux, brassières, and other articles for wear on the body or limbs where it is desired that a body of rubber in the fabric shall surround a part of the wearer's body, especially for reducing purposes, but not necessarily limited thereto. It is especially designed for those articles which are to serve the double purpose of reduction and perform the ordinary functions of such articles as above mentioned.

It has been proposed to manufacture articles of this general nature for similar purposes of pure rubber and also of certain fabrics rubberized. In the former case the rubber is affected by the perspiration and its life is very short as it soon gets into a condition in which it can be torn easily by the ordinary strains to which it is put in adjusting it and manipulating it after it is on. Even when new it is not strong enough.

In the case of the fabrics which have been rubberized by placing a layer of rubber on one side or inside there is little or no elasticity and one of the most important functions of the rubber itself is entirely lost. It retains odors also.

This invention is designed for the purpose of getting the full benefit of the rubber, both as a reducing agent and as an elastic agent, and yet providing such a strong article that it will wear as long as the ordinary non-elastic articles which have been on the market for many years. It also has a basis of textile material which permits of steels, whalebones, and other stiffening elements being permanently attached thereto without weakening it along the lines of attachment. The textile material is so made that sufficient spaces or interstices are provided to ensure the presence of rubber all the way through as well as on the surface.

One of the most important features of the invention is that, although the rubber in the goods is free to stretch, the extent of this stretch is limited, and therefore with a smaller amount of rubber, or rubber with less elasticity, all the elasticity that is necessary can be secured and yet the strength of the fabric is not decreased below that of the ordinary non-elastic fabrics which have been used. The fabric also is elastic in one direction only. This feature is very im-

portant because in the manufacture of a corset or the like from this fabric it can be arranged to have its direction of elasticity horizontal or circumferential and it can be stretched to any amount necessary without drawing it in at the top and bottom, and thus distorting its shape. Furthermore by having it entirely non-elastic in a vertical direction a fabric originally produced of the desired width will retain that width until the article is entirely worn out. In this way the shape of the original article is maintained, the necessary elasticity around the body is provided for, and the durability of the article is as great as that of any article of this character. The invention also involves the article made from this fabric.

Reference is to be had to the accompanying drawings, in which—

Fig. 1 is a side view of a corset constructed of fabric made in accordance with this invention;

Fig. 2 is a front view of a bandeau similarly made;

Fig. 3 is a diagrammatic transverse sectional view of a part of a machine for rubberizing the fabric after it is woven; and

Fig. 4 is a magnified view of a fabric, before it is rubberized, especially suitable for this purpose.

The fabric is woven, preferably of unbleached cotton, in the desired widths on looms which will weave elastic webbing but preferably provided with a leno, or double leno attachment. This woven elastic webbing is made with warps having interspersed among them additional threads in the nature of warp threads of elastic rubber. It is woven with the rubber threads in a stretched condition, and the warps of cotton, silk or other fibre are then necessarily contracted when the fabric has been produced and the strain is taken off the product so as to allow the rubber longitudinal threads to contract to substantially their natural length. The weaving is very loose so as to form large interstices in the fabric for a purpose that will appear hereinafter. I prefer to employ ordinary double leno weave which leaves the fabric *f* with interstices *g* as shown in Fig. 4. This fabric can be produced in any desired width and for the purpose of this invention it is made of the width required for the article to which it is to be applied, so that a single width of the goods ordinarily is used to form the article and the warp

100

95

100

105

110

and elastic rubber threads extend circumferentially or longitudinally. Such a fabric will stretch longitudinally without contracting laterally and it will not stretch laterally.

5 If a simple loosely woven or knitted fabric has been produced, the same is put under tension. This tension can vary in accordance with the conditions required, but we find that a tension of about 25% of the maximum 10 elongation of the fabric is a suitable amount. If a double leno fabric is used it need be put under only enough tension to hold it taut without wrinkling. The fabric *f* with covered or uncovered threads of rubber *r*, 15 preferably arranged in groups, is introduced between two rolls 10 and passed from between these rolls over another roll 11. Masses of rubber dough in a heated state are introduced between the rolls 10 and two 20 other rolls 12 so as to be rolled out by the two pairs of rolls, or latex is applied, and delivered on opposite sides of the fabric *f* between the two rolls 10. These rolls are heated to the proper temperature for vulcanization. The rubber is rolled through the interstices of the stretched fabric and simultaneously vulcanized. The rolls 10 are caused to press towards each other with a 25 high degree of pressure to consolidate the rubber as it is applied to the fabric. The result of this is to produce a rubberized fabric having not merely a coating of rubber on both sides but entirely filled with rubber and having the single integral mass of rubber 30 extending through to connect the rubber surfaces on both sides. It makes no difference in the completed fabric whether these threads are entirely bare and thus become entirely vulcanized to the other rubber 35 and lost therein, or whether they were originally wound with yarn and retain their identity. Their elasticity is substantially the same as the rubber *R* introduced. If it is desired to have a fabric with a smoother 40 surface on one side an additional layer of rubber can be applied in a similar manner.

45 After the rubberized fabric is delivered from the machine it has the characteristic that it will stretch longitudinally in the same direction as the rubber threads *r*, but not transversely, because the weft threads of the woven fabric have not been contracted or displaced in any way, and they prevent any stretching in that direction. The elasticity 50 in the longitudinal direction may not be as great as would be the elasticity of a pure rubber sheet of the same grade of rubber, if the rubber is applied to the woven fabric while the latter is in a stretched condition.

In either case the excessive elasticity of pure 60 rubber goods, which is a disadvantage, is overcome to the extent that may be necessary for the particular use to which the fabric is to be put.

The fabric thus produced is used in the 65 manufacture of corsets C as shown in Fig. 1, bandeaux B as shown in Fig. 2, hose supporters, surgical stockings, or any other desired article. Preferably it constitutes the entire article, except whatever binding 70 D is put on the edge, or stays E of any character which may be applied to it in the same manner as to a non-elastic woven fabric. It will be obvious that such stays, 75 bindings, and trimmings can be securely mounted on this fabric without injuring it, and without weakening the article at the points of juncture.

When the article is finished in this way 80 it furnishes a very durable construction having all the advantages of a pure rubber garment and yet it cannot be stretched out to such a point as to render it useless, and if the rubber does deteriorate from wear the rest of the garment holds together and performs its functions in a much better degree 85 than is the case with an all rubber garment. At the same time the elasticity is maintained which has not been done in the case of the 90 rubberized fabrics heretofore used for similar purposes. It can be washed off on both sides and thus kept in an odorless and sanitary condition.

Although we have illustrated and described only a small number of uses for 95 this product we are aware of the fact that it is capable of a wide extension of uses, and that any person skilled in the art can vary the weaving and construction of the fabric without departing from the scope of the 100 invention as expressed in the claim. Therefore, we do not wish to be limited in these respects, but what we do claim is:—

The method of making an elastic fabric 105 which consists in producing a loose textile fabric having elastic threads extending in one direction to give it elasticity in that direction, stretching said fabric longitudinally to a degree materially less than its elastic limit, and applying rubber to the 110 fabric and subjecting it to a high degree of pressure and temperature to vulcanize the rubber in position on the fabric and through it.

In testimony whereof we have hereunto 115 affixed our signatures.

ERNEST R. MILLS.  
CARL J. HAZELTON.